

## UNITED STATES PATENT OFFICE

2,368,158

METHOD OF TREATING CELLULOUSIC  
TEXTILE MATERIAL

Eric Owen Ridgway, Upper Montclair, and Frederick Curtis Tucker and Charles J. Kintner, Nutley, N. J., assignors to Ridbo Laboratories, Inc., a corporation of New Jersey

No Drawing. Application August 28, 1940,  
Serial No. 354,582

8 Claims. (Cl. 8—139)

This invention relates to the treatment of cellulosic textile material such as cotton, jute, linen and the like, preferably in the form of thread, yarn or woven material.

Among the primary objects of the invention is the chemical and physical treatment of cellulosic fibres which is relatively inexpensive, effective and easily controllable and adapted to produce a more readily absorbent and stronger textile fibre of substantially pure alpha cellulose from which the impurities have in large part been removed. The treatment greatly increases the tensile strength of the cellulosic material, to an extent far greater than that which would be expected by one skilled in the art; the tensile strength being increased approximately 20% and over above untreated gray goods and above goods treated according to the well-known mill methods of kiering, bleaching and mercerizing, or combinations thereof.

The improved method of treatment has the added advantage of being applicable to any continuous process of treating cellulosic material, such as mercerization, bleaching, or both; because our method is preferably carried out continuously.

The improved method comprises primarily two steps; the first step may be termed a "conditioning" step in that it partially removes impurities present in the cellulosic fibres, such as waxes, pectins and the lesser celluloses, and leaves the cellulosic textile material in the desired state for the second step of the method. The second step of the improved method comprises a combination of chemical and physical action on the cellulosic material, and it is during this step that the major proportion of the improvement in tensile strength, appearance and absorbency is obtained.

The first or "conditioning" step of the improved method can be partially performed by any of the well-known methods of kier boiling or bleaching or combinations thereof. However, we prefer to treat the cellulosic textile material in relatively high concentrations of sodium hydroxide or potassium hydroxide since we have found that this treatment is superior to the normal kier boil and can be completed in a relatively short time. After this treatment the materials are thoroughly washed in water to remove the hydroxide and are then ready for the second step of the process, which broadly comprises a plurality of immersions in a dilute water-soluble acid such as dilute sulphuric acid. Before the first bath and after each immersion the material is subjected to a mechanical squeezing action such as being forced through squeeze rolls.

In the first or conditioning step, the boiling sodium hydroxide preferably ranges in concentration from 12 to 96 grams sodium hydroxide per litre, and the material may be immersed in this solution at a boiling temperature for a period of from three minutes to two hours without deleterious action on the cellulosic fibres or any appreciably greater loss in weight, length or size of the yarn and thread than is now obtained in the well-known mill methods, although as mentioned the more dilute "kierboiling" concentrations may be employed with somewhat less satisfactory results. In commercial operations, the period of immersion in the boiling sodium hydroxide solution may be ten minutes, since further immersion produces improvements generally so small as not to be commercially feasible, except in such instances as when the material is so tightly packed in the vessel that the circulation of the solution is impaired and in such instances longer periods of immersion are desirable, although it is to be understood that longer immersion periods up to the limits expressed do not deleteriously affect the material being treated.

This first step in our improved method does not require the use of special equipment since it is not necessary that the material be treated under pressure unless a slight pressure is necessary to obtain thorough circulation of the treating solution throughout the material. For example, a kier, open tank or a Hussong machine may be employed; an injector type of kier, in which the solution is heated by live steam and circulated, has been satisfactorily employed since if the solution is at the boiling temperatures when the material is immersed, dilution caused by the steam is not appreciable.

The final stage in the first step of the method comprises washing the cellulosic material, preferably cotton, until substantially free of chemicals employed and the dissolved or partially dissolved impurities. It is preferred to wash the material with hot water since a thorough hot wash accentuates the partial bleaching effect produced by the boiling sodium hydroxide material. Before entering the second step of the improved method, the material should be cooled, preferably by means of a cold water bath.

After the preliminarily treated material has been thoroughly washed, it is ready for the second step of the method which, as previously mentioned, comprises a combination of chemical and physical action on the cellulosic material, and it is during the second step of the method that the

major improvement in tensile strength, appearance and absorbency is obtained.

The material is subjected to a plurality of treatments in a dilute solution of a water-soluble acid, organic or inorganic, or acid salt, preferably at room temperature. For example, sulphuric acid has been satisfactorily employed at concentrations varying from 3 grams to 70 grams per litre, and a typical satisfactory solution is that employing 38 grams per litre sulphuric acid. Before the first bath and between each succeeding bath, the material is passed through mechanical squeeze rolls which are set to obtain a 70% moisture retention, or lower, and may be preferably maintained to secure approximately 50% retention or lower. A thorough squeeze of the material, such as obtained by the moisture retentions indicated, is quite important to obtain the desired result. The cellulosic material need only be immersed in the acid solution long enough to completely saturate all of the fibres, although the time may be varied depending upon whether the material being treated is in the form of cloth, yarn, thread or fibres; there is no deleterious effect on the material over a relatively longer period of immersion as long as the material is completely submerged in the solution. The concentration of the acid bath may be increased slightly with each succeeding bath.

As previously mentioned, the squeeze rolls should be set to give a residual moisture retention of less than 70% of the weight of the dry cellulosic material being treated, and to obtain the best results it is essential that the residual moisture retention should be 50% or under. The importance of the tightness of the mechanical squeeze rolls through which the cellulosic material is run before and after saturation in a plurality of dilute acid baths, is illustrated by the improvement obtained in cotton thread so treated. It has been found that where the squeeze rolls are set to give over 70% retention of the solution in the fibres, practically no increase in tensile strength is obtained, whereas up to and beyond 20% tensile strength improvement is obtained when the squeeze rolls are set so that the solution retention in the fibres is lowered below 70%. Accordingly, it will be understood that while the pretreatment of the textile material may be varied as previously set forth, and while various water-soluble acids and concentrations thereof may be employed to obtain satisfactory results, it is essential that the material be squeezed to the extent indicated before the first bath and after each immersion in the acid bath.

The number of acid baths preferably ranges from four to ten and, for most materials, the desired results are obtained after a total of seven squeezes and six immersions in the acid solution. For example, with this number of physical and chemical treatments, it has been found that the tensile strength of the material is increased approximately 20%. Some improvement has been obtained by the use of two acid baths, the material being squeezed in the manner mentioned before, between and after the baths. However, since it has been found that the tensile strength increases with a greater number of consecutive acid baths with squeezes between each bath and after the final bath, a greater number of consecutive acid baths is preferred. The improvement after ten consecutive baths and eleven squeezes of the type described is not of great importance, although there is some purification of the fibrous structure up to ten baths.

The acid and squeezing treatment may be performed with relatively simple apparatus, for example, a single acid chamber may be employed over which are mounted seven sets of squeeze rolls of the type described so arranged that the cellulosic textile material will receive six saturations in the dilute acid solution with a mechanical squeeze of the nature described before the first immersion and between each subsequent immersion and after the final bath. The use of a centrifuge or other drying apparatus to reduce the residual moisture content of the treated material to 70% or under in place of the squeeze rolls is not particularly recommended, although fairly satisfactory results may be so obtained, since the same measure of control cannot be obtained and the same measure of uniformity or consistency in results has not been obtained.

As an example of the method of treatment, the following is given as a typical example of treating yarn or thread. It is preferred that such material should be treated in the warp form rather than in the form of large skeins.

One pound of cotton yarn or thread is boiled for ten minutes at atmospheric pressure in 4 litres of 64 grams of sodium hydroxide per litre. The material is then washed thoroughly with hot water until it is substantially free of alkali and is then cooled by washing in cold water.

The material is then run through squeeze rolls of the type described, which are set to retain approximately 50% of the residual moisture to the dry weight of the material. The thread or yarn is then saturated in an acid bath comprising 38 grams of sulphuric acid per litre. The material is then again passed through squeeze rolls set to obtain the low moisture content described. This action is repeated until the material has been saturated in the dilute acid bath six times and has been squeezed after each bath. The material is then washed in water until free of acid, and dried.

What we claim is:

1. The method of treating natural cellulosic textile materials, comprising treating said materials in a hot, caustic alkali solution, washing said material to remove said alkali solution and then treating said materials in a plurality of at least four dilute baths of a water-soluble acid, said material being partially dried by mechanical means to a moisture retention under 70% of the weight of the dry textile material before said first bath and between each succeeding bath and after the final bath.
2. The method of treating natural cellulosic textile material, comprising immersing said material in a boiling concentrated caustic alkali bath of at least 12 grams sodium hydroxide per litre, washing said material to remove the caustic alkali solution, and then treating said material at least six times in a dilute bath of a water-soluble acid, said material being partially dried to a moisture retention under 70% of the weight of the dry textile material by mechanical means before the first bath, between each succeeding bath, and after the final bath.
3. The method of treating natural cellulosic textile material after it has been kier boiled, comprising washing said material in water and then squeezing said material to an expression under 70% moisture retention calculated on the weight of the dry textile material, immersing said material in a dilute bath of a water-soluble acid, again squeezing the material to a moisture retention of under 70%, and repeating the sat-

uration of said material in the dilute water-soluble acid bath and the squeezing action to the moisture retention specified at least three times.

4. In a method of treating natural cellulosic textile material, the successive steps of bleaching, washing said material in water, subjecting the material to the mechanical squeezing of a character to obtain under 70% retention of the residual liquid to the dry weight of the cellulosic textile material, saturating said material in a dilute bath of a water-soluble acid, then squeezing said material in the manner above defined to obtain under 70% retention of the residual liquid to the dry weight of the cellulosic textile material, and repeating at least three times the saturation of said material in the dilute acid bath and the squeezing to obtain under 70% retention of the residual liquid to the dry weight of the cellulosic textile material.

5. The method of treating natural cellulosic textile material to improve its tensile strength and absorbency, comprising immersing said material in a caustic solution at approximately the boiling temperature for upwardly of three minutes, washing said material to remove said caustic solution, partially drying said material by mechanically squeezing it to reduce the residual liquid to under 70% of the dry weight of the cellulosic textile material, and then thoroughly saturating said material at least six successive times in a solution of sulphuric acid containing from 3 to 70 grams sulphuric acid per litre, said material being partially dried by squeezing it to reduce the residual liquid to under 70% of the dry weight of the cellulosic textile material between each bath and after the last bath.

6. The method of treating natural cellulosic textile materials to improve their tensile strength and absorbency, comprising immersing said ma-

terial in a hot, caustic solution of at least 12 grams caustic material per litre for at least three minutes, washing said material to remove said caustic alkali solution, and then treating said materials in a series of at least four dilute aqueous baths of a water-soluble acid, said materials being squeezed in a manner, to obtain a moisture retention of approximately 50% of the weight of the dry cellulosic materials, before the first bath and after each succeeding bath.

7. In a method of treating natural cellulosic textile materials to improve their tensile strength and absorbency, the steps comprising first pre-treating in a concentrated caustic solution said material to remove impurities and then thoroughly saturating said material at least six successive times in a solution of sulphuric acid containing from 3 to 70 grams sulphuric acid per litre, said materials being squeezed after each bath in a manner to dry the material to a retention of residual liquid of approximately 50% of the dry weight of the cellulosic textile material.

8. The method of treating natural cellulosic textile materials to improve their tensile strength and absorbency, comprising immersing said material in a boiling caustic solution of at least 12 grams caustic material per liter for at least 3 minutes, washing said material to remove caustic alkali solution therefrom, and then treating said materials in a series of at least 4 dilute aqueous baths of a water-soluble acid, said materials being squeezed in a manner to obtain a moisture retention of under 70% of the weight of the dry cellulosic materials, the material being squeezed at least 5 times and the treatment in the acid baths and the squeezings being alternated.

ERIC OWEN RIDGWAY.

FREDERICK CURTIS TUCKER.

CHARLES J. KINTNER.